

## UNITED STATES PATENT OFFICE

HARRY T. BENNETT, OF TULSA, OKLAHOMA

## PROCESS OF TREATING CRUDE PETROLEUM

No Drawing.

Application filed July 22, 1926. Serial No. 124,300.

This invention relates to improvements in the treating of crude petroleum, and particularly to the treatment of crude petroleum for improving the flowing ability at low temperatures. It comprises a process for treatment of crude petroleum with a soap of such character and amount that the crude petroleum which would ordinarily be solid at low temperatures is rendered fluid.

Crude petroleum varies in composition and physical properties depending on the origin. Some crudes flow readily at 0° F. while others become solid at relatively low temperatures. For example, a crude such as that from the Amarilla field is solid at 60° F. or below. Purchasers and producers are frequently confronted with a difficult problem of handling such a crude which has become solid at low temperatures. The usual methods heretofore were to heat the crude until the wax or other solid material becomes melted or to dilute the solid crude with a more fluid sample.

I have discovered that crude petroleum can be rendered fluid and retained in a fluid condition by the addition of a small quantity of soap. The nature and quantity of the soap depends upon the properties of the crude petroleum, and to obtain the best results these factors may be accurately ascertained by experiments.

In practicing my invention the crude petroleum may be treated cold or hot, preferably hot, with a desired quantity of the given soap, the soap being thoroughly incorporated into the oil. Or, a better method is to first commingle the soap with a vehicle comprising a suitable quantity of a hot or cold carrier (such as a petroleum product having a higher initial boiling point than the crude), the resulting product then incorporated with the crude petroleum to be treated.

In actual operation I have treated an Amarilla crude petroleum which became solid at 60° F. with 0.1 per cent aluminum stearate and thus rendered it capable of flowing at temperatures as low as 0° F. Approximately the same results have been obtained by using iron or zinc soaps instead of aluminum stearate.

Without quoting further examples here, I will point out the flexibility of the invention and, instead of limiting myself to specific soaps, include all soaps of the nature of the above, whether they be mono, di, or tri-basic and whether produced by the saponification of an animal or vegetable fatty acid. It is also understood that I do not limit myself to a specific amount of soap, for this varies with the nature of the crude petroleum and the character of the soap.

Also, I do not limit myself to crude petroleum in the sense that it is the crude oil as received from the ground, but, in certain cases, the crude petroleum may become weathered in storage or by partial distillation (sometimes called topped crude petroleum), so that in the following claims the term "crude petroleum" will be used as embracing the entire class as herein described.

Recognized procedure for determining pour points is provided in Technical Paper 3238, U. S. Government Specification No. 2d, Department of Commerce Publication, U. S. Government Master Specification for Lubricants and Liquid Fuels and Methods for Sampling and Testing, on pages 40 and 41 of which is set forth procedure for pour point.

I claim:

1. The process which comprises lowering the pour point of crude petroleum by commingling with said crude petroleum, a minute quantity of soap capable of lowering the pour point of the oil in amount sufficiently low to render the product capable of flowing at low temperatures without substantially affecting the viscosity of the petroleum.

2. The process which comprises lowering the pour point of crude petroleum by commingling with the crude petroleum a minute quantity of aluminum stearate in amount sufficiently low to render the product capable of flowing at low temperatures without substantially affecting the viscosity of the petroleum.

3. The process which comprises lowering the pour point of crude petroleum by commingling with the crude petroleum a quantity of aluminum soap capable of lowering the pour point of the oil about .1 per cent by

weight of the crude petroleum and thereby rendering the product capable of flowing at low temperatures without substantially affecting the viscosity of the petroleum.

5 4. The process which comprises lowering the pour point of crude petroleum of a type which becomes solid at 60° F. by commingling with said crude petroleum approximately 0.1% by weight of a metal soap  
10 capable of lowering the pour point of the oil and thereby rendering the product capable of flowing at 0° F.

5. The process which comprises lowering the pour point of crude petroleum by commingling with said crude petroleum a minute quantity of a metal soap capable of lowering the pour point of the oil in amount sufficiently low to render the product capable of flowing at low temperatures without substantially  
20 affecting the viscosity of the oil.

In testimony that I claim the foregoing I  
hereunto affix my signature.

HARRY T. BENNETT.

25

30

35

40

45

50

55

60

65